

## UNITED STATES PATENT OFFICE.

GUIDO BONADÉ BOTTINO, OF TURIN, ITALY, ASSIGNOR TO A. G. E. D. SOCIETÀ ANONIMA ARTI GRAFICHE & DECORATIVE, OF TURIN, ITALY.

## PROCESS FOR TRANSFERRING DESIGNS.

No Drawing.

Application filed April 1, 1924. Serial No. 703,525.

To all whom it may concern:

Be it known that I, GUIDO BONADÉ BOTTINO, a subject of the King of Italy, resident of 4 Via Fabro, Turin, in the Kingdom of Italy, and whose post-office address is 4 Via Fabro, Turin (3), Italy, have invented certain new and useful Improvements in Processes for Transferring Designs; and I do hereby declare the following to be a full, clear, and exact description of the invention, such as will enable others skilled in the art to which it appertains to make and use the same.

This invention relates to a method of printing drawings or inscriptions and transferring them in an indelible manner in the heat on wood, cloth, and other materials.

The invention comprises the preparation of the varnishes adapted to be used in ordinary printing machines and transferred, under the action of heat, from the printed sheets of paper on wood, cloth, etc., and the transfer process.

In order to prepare the varnish, the colours or dyes (metallic oxides) are added to a mixture previously prepared in the heat of wax and paraffin dissolved in turpentine with the addition of a suitable quantity of colophony.

The following is an example of the constituents used in preparing the varnish:

About 300 grams of wax.

About 50 grams of paraffin.

1 liter of turpentine.

400 grams of colophony.

The quantity of colour added to the mixture varies with the more or less oily consistency of the colour.

The paper on which the designs to be transferred are printed shall be well sized and of strong fibre so as not to absorb an excessive amount of varnish.

In order to square off and pile up the printed sheets, these must be dried so as to avoid any smutting or blurring.

To this effect the sheets, once printed, are subjected to a very fine spray of colophony.

The process of transferring on wood, cloth, etc., the designs or inscriptions printed in the above mentioned manner consists in previously moistening the sheet, this being conveniently done by laying it on the surface of the water in a container with the printed side turned upwards. The design is then transferred by compressing the print against the desired surface by means of a hot press.

When the surface is a porous one (as in the case of wood, cloth, etc.) the special varnish related to above penetrates it indelibly in such manner that it shall not be effaced or blotted out. The same varnish applied on glass, metal, etc. adheres permanently thereto.

The above noted proportions of the varnish constituents can be varied, and some of the substances can be replaced by others having similar properties without departing from the spirit of the invention.

What I claim is:

1. Process for printing designs and transferring them on wood, cloth, etc., characterized by the fact that the varnishes employed in the preparation or printing of the design consist of colours (metallic oxides) with a mixture of wax and paraffin dissolved in turpentine to which is added colophony, such varnishes being used in ordinary printing machines for printing the design to be transferred.

2. Process as claimed in claim 1, characterized by the fact that the printed design is pulverized with finely subdivided colophony in order to dry the prints and to allow squaring off and piling up of the sheets.

3. Process as claimed in claims 1 and 2, wherein the printed design is first moistened and then compressed against the surface to which it is to be transferred by means of a hot press.

In testimony that I claim the foregoing as my invention, I have signed my name.

GUIDO BONADÉ BOTTINO.